

Feb. 20, 1968

T. C. McGEARY ETAL

3,369,386

WIRE DRAWING APPARATUS

Original Filed Nov. 2, 1964



INVENTORS  
THOMAS C. McGEARY  
LEWIS M. COWDEN  
BY *Barnwell P. King*  
ATTORNEY

## 1

3,369,386

## WIRE DRAWING APPARATUS

Thomas C. McGahey and Lewis M. Cowden, Indianapolis, Ind., assignors to Union Carbide Corporation, a corporation of New York

Continuation of abandoned application Ser. No. 408,279, Nov. 2, 1964. This application Mar. 13, 1967, Ser. No. 622,826

5 Claims. (Cl. 72—289)

This invention relates to wire drawing apparatus, and more particularly, to wire contact members, such as draw blocks.

Briefly, the invention provides a wire drawing apparatus comprising, for example, a metal draw block having an outer coating of refractory material the minimum thickness of which is 0.010 inch, a hardness of between 800 and 1,300 V.P.N., and a micro-lamellar structure.

This application is a continuation of application Ser. No. 408,279, filed Nov. 2, 1964, now abandoned.

In the manufacture of wire, that is, in the drawing of wire down to its required size, draw blocks are used to pull the wire through the dies. Such draw blocks, or as they are sometimes called, capstans, undergo severe wear and abrasion. Such wear, caused by the thin wire traveling at high speed, forms thin grooves in the surface which lead to jamming and breaking of the wire strands. In addition to the wear problem, there is also a corrosion problem due to the lubricant being used in the drawing operation.

Prior to this invention, wire drawing blocks primarily consisted of flame hardened cast iron. Normal service life with such draw blocks amounted to about six months. Of recent years attempts have been made to increase the life of draw blocks by applying a wear resistant coating to the wear surface. A hard wear resistant bonded tungsten carbide coating has been used, for example. While such coating measureably increased the life of the draw blocks, it still has not met the heavy demands of the industry.

It is, therefore, the principal object of the present invention to provide an improved wire contact member for wire drawing machines, which will give a longer service life than has been possible in the past.

FIGURE 1 is a plan view of an example of wire drawing apparatus incorporating the invention;

FIGURE 2 is an enlarged view in side elevation of the draw block;

FIGURE 3 is a view similar to FIGURE 1 of a modification of the invention;

FIGURE 4 is an enlarged perspective view in cross section of one of the draw blocks shown in FIGURE 3; and

FIGURE 5 is a fragmentary enlarged view in cross section of a portion of the block shown in FIGURE 2.

With reference to FIGURE 1, there is depicted a draw block 14 for one type of wire drawing operation. Wire 10 is drawn from a supply reel 11 through a die 12 by a draw block 14 driven by a motor 15, FIGURE 2. From there the wire 10 is fed to and wound on a reel 16. The function of the draw block 14 is to pull the wire 10 through the preceding die 12. In this type of operation a straight frusto-conically faced draw block 14 is used. The wire 10 climbs up the tapered face 13 of the block 14, as shown.

Another type of wire drawing operation is schematically shown in FIGURE 3. In this system, the wire 10 is pulled through separate dies encased in housing 32 by stepped draw blocks 30. The wire is pulled from step 1 through a die to step 1a, then from step 1a through another die to step 2, and so on. In this system, each draw block 30 is not only stepped, but each step is grooved at 34 as shown in FIGURE 4.

## 2

Such pulling of the wire by the draw blocks in both systems, presents a severe wear problem, especially when the speed with which the wire is traveling over the blocks is considered, such speed being as high as 5000 ft./min.

5 According to the invention, the outer surface of the draw blocks 14 and 34 are provided with a novel coating 18, FIGURE 5, composed of refractory material selected from the class consisting of chrome oxide, and ferrochrome-tungsten carbide alloy. More particularly, powder of the selected material is passed through an arc torch in the manner described in U.S. 3,016,447 and then, for example, projected onto a base, which in the case of the present invention would be the outer surface of the wire contact member. Because of the torch's constricting nozzle, the arc becomes well stabilized thus yielding an intense columnar plasma. The torch itself operates in a non-transferred mode. Coatings formed according to this arc process have a dense, micro-lamellar structure with bonded, overlapping leaves.

10 According to the invention, the outer surface of the draw blocks 14 and 34 are provided with a novel coating 18, FIGURE 5, composed of refractory material selected from the class consisting of chrome oxide, and ferrochrome-tungsten carbide alloy. More particularly, powder of the selected material is passed through an arc torch in the manner described in U.S. 3,016,447 and then, for example, projected onto a base, which in the case of the present invention would be the outer surface of the wire contact member. Because of the torch's constricting nozzle, the arc becomes well stabilized thus yielding an intense columnar plasma. The torch itself operates in a non-transferred mode. Coatings formed according to this arc process have a dense, micro-lamellar structure with bonded, overlapping leaves.

15 According to the invention, the outer surface of the draw blocks 14 and 34 are provided with a novel coating 18, FIGURE 5, composed of refractory material selected from the class consisting of chrome oxide, and ferrochrome-tungsten carbide alloy. More particularly, powder of the selected material is passed through an arc torch in the manner described in U.S. 3,016,447 and then, for example, projected onto a base, which in the case of the present invention would be the outer surface of the wire contact member. Because of the torch's constricting nozzle, the arc becomes well stabilized thus yielding an intense columnar plasma. The torch itself operates in a non-transferred mode. Coatings formed according to this arc process have a dense, micro-lamellar structure with bonded, overlapping leaves.

20 According to the invention, the outer surface of the draw blocks 14 and 34 are provided with a novel coating 18, FIGURE 5, composed of refractory material selected from the class consisting of chrome oxide, and ferrochrome-tungsten carbide alloy. More particularly, powder of the selected material is passed through an arc torch in the manner described in U.S. 3,016,447 and then, for example, projected onto a base, which in the case of the present invention would be the outer surface of the wire contact member. Because of the torch's constricting nozzle, the arc becomes well stabilized thus yielding an intense columnar plasma. The torch itself operates in a non-transferred mode. Coatings formed according to this arc process have a dense, micro-lamellar structure with bonded, overlapping leaves.

25 According to the invention, the outer surface of the draw blocks 14 and 34 are provided with a novel coating 18, FIGURE 5, composed of refractory material selected from the class consisting of chrome oxide, and ferrochrome-tungsten carbide alloy. More particularly, powder of the selected material is passed through an arc torch in the manner described in U.S. 3,016,447 and then, for example, projected onto a base, which in the case of the present invention would be the outer surface of the wire contact member. Because of the torch's constricting nozzle, the arc becomes well stabilized thus yielding an intense columnar plasma. The torch itself operates in a non-transferred mode. Coatings formed according to this arc process have a dense, micro-lamellar structure with bonded, overlapping leaves.

30 According to the invention, the outer surface of the draw blocks 14 and 34 are provided with a novel coating 18, FIGURE 5, composed of refractory material selected from the class consisting of chrome oxide, and ferrochrome-tungsten carbide alloy. More particularly, powder of the selected material is passed through an arc torch in the manner described in U.S. 3,016,447 and then, for example, projected onto a base, which in the case of the present invention would be the outer surface of the wire contact member. Because of the torch's constricting nozzle, the arc becomes well stabilized thus yielding an intense columnar plasma. The torch itself operates in a non-transferred mode. Coatings formed according to this arc process have a dense, micro-lamellar structure with bonded, overlapping leaves.

35 According to the invention, the outer surface of the draw blocks 14 and 34 are provided with a novel coating 18, FIGURE 5, composed of refractory material selected from the class consisting of chrome oxide, and ferrochrome-tungsten carbide alloy. More particularly, powder of the selected material is passed through an arc torch in the manner described in U.S. 3,016,447 and then, for example, projected onto a base, which in the case of the present invention would be the outer surface of the wire contact member. Because of the torch's constricting nozzle, the arc becomes well stabilized thus yielding an intense columnar plasma. The torch itself operates in a non-transferred mode. Coatings formed according to this arc process have a dense, micro-lamellar structure with bonded, overlapping leaves.

| 40 | Wear Surface Material              | Vickers Hardness | Time Before Grooves Appeared | Type of Wire Drawn   |
|----|------------------------------------|------------------|------------------------------|----------------------|
|    | Flame Hardened                     | 700              | 7 months                     | Steel.               |
|    | Aluminum oxide                     | 1,000            | 1 month                      | Copper based alloys. |
| 45 | Tungsten Carbide (bonded)          | 1,400            | 3-4 months                   | Steel.               |
|    | Chrome oxide                       | 1,300            | Over 20 months               | Do.                  |
|    | Ferrochrome-tungsten carbide alloy | 900              | Over 14 months               | Do.                  |

## Example 1

50 A carbon steel draw block of the type described with reference to FIGURE 2 was coated. The draw block had a height of about 5" and an O.D. of 20". The torch was held about  $\frac{3}{4}$  to 1 inch away from the coating surface. The draw block was rotated at about 300 r.p.m. Argon gas was fed through the torch at the rate of about 300 c.f.h. Powdered chrome oxide was fed through the torch with the aid of argon gas at the rate of 50-60 gms. per min. The substrate was cooled with carbon dioxide. A coating about .010 inch thick was obtained.

## Example 2

55 Five nine-step, carbon steel draw blocks of the type shown in FIGURE 4 were coated by the same process. The blocks had a 10 inch O.D. at the top. The grooves were  $\frac{1}{8}$  inch deep by about  $\frac{1}{2}$  inch wide. Argon gas was fed through the torch along with the chromia powder which was also carried by argon. The blocks were cooled with carbon dioxide. Coating was achieved three steps at a time, starting with the step at the largest diameter. The torch standoff was maintained at about  $1\frac{1}{2}$  inches in all cases. During the first six steps the draw blocks were ro-

lated at about 760 r.p.m., during the last three steps, at 2080 r.p.m. The coating thickness varied from .010 to .014 inch.

After the draw blocks were coated, they were finished by one of three procedures depending upon the size of the wire to be drawn: sanding, grinding, or grinding and lapping. For example, for a  $\frac{3}{8}$  inch wire, the surface was sanded only. While for a .010 inch wire, the surface was ground and lapped.

The preferred ferrochrome-tungsten carbide alloy is disclosed in the application of Ronald H. Rath, Ser. No. 336,353, filed Jan. 8, 1964, for Wear and Corrosion Resistant Coating.

*Example 3*

A carbon steel draw block of the type described with reference to FIGURE 2 was coated with an arc torch by the process described. The draw block had a height of about 12" and an O.D. of 24". The torch was held about  $\frac{3}{16}$  to  $1\frac{3}{16}$  inch away from the coating surface. The draw-block was rotated at about 340 r.p.m. Argon gas and nitrogen gas were fed through the torch at the rate of about 330 c.f.h. Powdered 40% ferrochrome-60% tungsten carbide powder was fed through the torch with the aid of argon gas at the rate of 68 grams per min. A coating about .011 inch thick was obtained.

We claim:

1. Wire drawing apparatus comprising a metal draw

block having an outer coating of refractory material the minimum thickness of which is 0.010 inch, a hardness of between 850 and 1,300 V.P.N., and a micro-lamellar structure.

5 2. Wire drawing apparatus as defined by claim 1, in which the refractory coating material is selected from the class consisting of chromia and ferrochrome tungsten carbide alloy.

3. A wire draw block composed of steel having a wire contacting surface coating consisting of chromia.

4. A wire draw block composed of steel having a wire contacting surface coating consisting of ferrochrome-tungsten carbide alloy.

15 5. Wire drawing apparatus comprising a member provided with a coating adapted for contact with moving wire, said member being composed of metal and the coating thereon being composed of a lamellar structure of refractory material selected from the class consisting of chromia and a ferrochrome-tungsten alloy.

20

**References Cited**

**UNITED STATES PATENTS**

2,025,535 12/1935 Sommer ----- 72—419

25 CHARLES W. LANHAM, *Primary Examiner*.

H. D. HOINKES, *Assistant Examiner*.